

# UNITED STATES PATENT OFFICE.

JOSEPH BRUECK, OF NEW YORK, N. Y.

## NAIL-POLISH.

1,388,546.

Specification of Letters Patent. Patented Aug. 23, 1921.

No Drawing.

Application filed September 3, 1919. Serial No. 321,446.

*To all whom it may concern:*

Be it known that I, JOSEPH BRUECK, a citizen of the United States of America, residing in the city of New York, borough of Bronx, county of Bronx, and State of New York, have invented certain new and useful Improvements in Nail-Polishes, of which the following is a full, clear, and exact description.

- 10 My invention is a nail polish, and contemplates the production of a nail polish in the form of a rather thin, syrup-like liquid, which is applied to the nails by aid of a brush in order to polish the nails.
- 15 I mix together four gallons of acetone and one gallon of amyl acetate, and then add thirty two ounces of gun cotton, which is readily soluble in the mixture. The gun cotton disappears in a few hours. The mixture
- 20 is now stirred, and appears in the form of a thin liquid having a syrup-like consistency.

The liquid is now set aside and allowed to stand for a few weeks, during which time it gradually becomes clear. Then I add four ounces of alkanet as a coloring.

25 The material thus prepared is well adapted for manicuring and is easily applied to the nails, after which they may by gentle rubbing be given a high polish.

Having thus described my invention, what I claim as new and desire to secure by United States Letters Patent is:

- 30 1. A nail polish containing acetone and amyl acetate, and gun cotton dissolved therein.
- 35 2. A nail polish comprising the following ingredients in the proportions stated: acetone four gallons, amyl acetate one gallon, gun cotton thirty-two ounces, and alkanet root approximately four ounces.

JOSEPH BRUECK.